

1

3,297,553

## ELECTROLYTIC PRODUCTION OF TUNGSTEN AND MOLYBDENUM

Harvey L. Slatin, New York, N.Y., assignor to Timax  
Associates, New York, N.Y., a partnership of New  
York

No Drawing. Filed May 28, 1963, Ser. No. 283,697  
6 Claims. (Cl. 204—64)

This invention relates to the production of tungsten and molybdenum directly from crude concentrates by fusion electrolysis.

In my Patent No. 2,960,451 entitled, "Electrolytic Production of Refractory Multivalent Metals," a method for producing high purity tungsten or molybdenum is disclosed by electrolyzing tungsten anhydride ( $WO_3$ ) or molybdc oxide dissolved in a fused bath containing alkaline earth metal halides, such as calcium chloride ( $CaCl_2$ ), and alkaline earth metal oxides, such as calcium oxide ( $CaO$ ). When scheelite ( $CaWO_4$ ) or powellite ( $CaMoO_4$ ) is used in place of the tungsten anhydride or molybdc oxide as feed material, no calcium oxide is required since scheelite and powellite already contain the required calcium oxide.

In carrying out this latter embodiment of the process, the crude scheelite, powellite or processed molybdenum ores may be supplied directly to the electrolyte with a tungsten or molybdenum deposit of over 99% purity being obtained from the electrolyte. The metallic contaminants, such as iron or molybdenum which are usually in high concentration in the crude scheelite concentrate feed, appear in minor traces or in greatly reduced proportion in the deposit.

In continuous processing the concentration of calcium oxide in the electrolyte builds up as more and more scheelite or processed powellite concentrate is added to replenish the depleted tungsten or molybdenum. As the concentration of excess calcium oxide increases in the electrolyte, the quality of the electrodeposition process seems to be impaired so that the recovery efficiency falls off and the purity of the deposit decreases. As described in my Patent No. 2,960,451 the concentration of the alkaline earth metal oxide may be in the range from below 5 weight percent to 40 and over with effective results. The preferred concentrations are in the order of 10–20% by weight and are related to the  $WO_3$  concentration.

The primary object of this invention is to improve the process so that consistently high purity tungsten or molybdenum may be produced with high recovery efficiency in the fusion electrolysis of crude ore concentrate and calcium chloride electrolyte.

Another object of this invention is to provide a means for maintaining the electrolyte in such condition that the crystal size of the deposited tungsten or molybdenum remains large; the color of the deposit is silvery; the metal is substantially free of "bronzes," lower oxides, carbides, borides, phosphides, silicides, sulfides, selenides, arsenides or the like.

These and other objects are realized by the invention by periodically converting the excess calcium oxide which builds up in the electrolyte to calcium chloride, which is the principal ingredient of the bath. This purpose may be attained in many ways, but it is preferable to bubble chlorine gas through the bath. By doing this periodically either before or after or during the addition of the ore, the electrolyte is sustained in such condition so as to maintain continued operation of the process.

The term high purity metal as used herein refers to metal whose purity lies above 99%.

The improvement embodied by the instant invention may better be understood by considering the following illustrations of my invention.

The electrolytic cell used in the following examples

2

was made of graphite set in a welded shell crucible made of "Inconel." The cell was 10" O.D. and 8" I.D. and 14" tall, inside height. The cell was not sealed airtight but the cathode electrodeposit was allowed to cool in a cylinder surrounding the cathode through which helium gas was passed, thus effectively isolating the cathode from air and other gaseous contaminants. The electrolytic cell was made the anode to a depended cathode centrally located in the graphite crucible. The fused salt depth was about 10 inches with about 7" of cathode immersion. The cathode in these runs was an AGS-X grade graphite rod having an outside diameter of two inches and a length of three feet.

The cell assembly was placed in an electrically heated furnace which was thermostatically controlled. The direct current was supplied by a voltage adjustable rectifier.

The raw material feed was crude mill concentrate scheelite having the following petrographic analysis:

|               | Vol. percent |
|---------------|--------------|
| 20 Pyrohotite |              |
| Garnet        |              |
| Actinolite    |              |
| Epidote       |              |
| Chloride      |              |
| 25 Scheelite  | 85           |

Chemical analysis:

|                  | Percent by wt. |
|------------------|----------------|
| WO <sub>3</sub>  | 69.5           |
| Fe               | 3.1            |
| Mo               | 1.2            |
| Mn               | 1.4            |
| Ca               | 17.2           |
| CO <sub>2</sub>  | 0.2            |
| Cu               | 0.027          |
| Sr               | 0.012          |
| Zr               | 0.063          |
| Cb               | 0.015          |
| SiO <sub>2</sub> | N.A.           |

40 The solute was anhydrous calcium chloride weighing about 33 lbs. which was fused to a clear water-white melt. Sufficient scheelite concentrate was added to provide a 5 to 10% by weight solution calculated as tungsten. This concentration appeared to give the best results. At higher concentrations scheelite crystallizes out and may interfere physically. The bath depth is about 10".

45 The operating procedure is as follows. A 2" O.D. graphite rod, acting as cathode, is lowered into the molten bath for an immersion of seven inches. The current is adjusted to the selected cathode current density based on the 2" O.D. x 7" immersion. A cathode that has been previously used in the electrolysis of tungsten is preferred, since in such use a thin film is produced which adheres tenaciously to the electrode and facilitates the adherence of subsequent electrodeposits.

50 The electrolysis is continued at the temperature set for 4 hours. Then the cathode with its electrodeposit and still under impressed D.C. voltage is slowly withdrawn from the bath and retained in the cell. The fluid salts are allowed to drain back into the bath. During this time a clamshell-like steel cylinder surrounds the cathode through which helium or other inert gas may be passed to form an inert atmosphere around the deposit.

55 After the cathode has cooled sufficiently to be handled, it is detached from the cathode holder and another electrode is put in its place. The electrolysis is recommenced.

60 The electrodeposit is stripped from the cathode and introduced into a container having a mechanical agitator such as a "Lightning" stirrer and a water inlet and weir overflow. In a few minutes the electrodeposited mass disintegrates as the soluble salts are washed away. Since the cell is not airtight, carbonates may form in the elec-

trolyte. These are easily decomposed by HCl solution to facilitate the washing. Further aid to cleaning up the metal deposit may comprise treating with caustic soda solution and the like. When the metal is saltfree by test for chloride ion, the deposited metal is transferred to a filter and air dried.

The dried metal is silvery in color. It is classified as to particle size and analyzed for blending or other desired purpose.

The calcium oxide in the bath may be combined in complexes with the tungstic oxide in the form of scheelite or may be separate in the bath. The calcium oxide in the bath separate from the complexes is known as a free calcium oxide, since it is free of the tungstic oxide. In the present process the free calcium oxide is maintained between about 0.1% and 15%.

The results of four runs operated as stated above are tabulated below.

TABLE I

Duration of Run: 4 hrs. each (2 runs mixed).  
 Temperature of Electrolyte: 1,000° C.  
 Bath Conc.: 10% W in  $\text{CaCl}_2$  (feed scheelite concentrate).  
 Voltage: 2.4 V.  
 Current: 150 amps.  
 Cathode current density: 3.5 amps./in.<sup>2</sup> initial.

|                     |                       |                       |         |         |         |
|---------------------|-----------------------|-----------------------|---------|---------|---------|
| Screen Analysis:    |                       |                       |         |         |         |
| Size                | +100                  | +150                  | +200    | +325    | -325    |
| Wt. %               | 1.0                   | 4.9                   | 61.2    | 32.9    | 32.9    |
| Chem. Analysis, W % | 93.2                  | 95.5                  | 99.0    | 98.9    | 98.9    |
| Major Impurities    | Brick, Fe, C          | Brick, Fe, C          | Mo .019 | Mo .019 | Mo .019 |
| X-ray Impurities    | <.01 W <sup>2</sup> C | <.01 W <sup>2</sup> C | Fe <.5  | Fe <.5  | Fe <.5  |
|                     | .3 scheelite          | .2 scheelite          | None    | None    | None    |

Each day or as required five pounds or more of scheelite concentrate is added to the electrolyte to replenish the depleted tungsten. I have found that by blowing dry chlorine gas through an inert tube made of quartz or "Sillimanite" towards the bottom of the cell at a rate so that the bath is well stirred by the gas bubbles and

The brick originated from improper handling of the furnace cover. The carbon appears through mechanical abrasion and the scheelite through mechanical entrainment. Much of the iron may be attributed to corrosion of the shell lining. With reasonable care and proper cell design, such extraneous impurities do not appear.

TABLE II

Duration of Run: 4 hrs. each (2 runs mixed).  
 Cathode: 2" Dia. graphite rod 7" immersion.  
 Temperature of Electrolyte: 1,000° C.  
 Bath: 10" depth containing 10% by wt. W in  $\text{CaCl}_2$ .  
 Anode: Cell crucible (graphite).  
 Voltage: 2.2 volts.  
 Current: 150 amperes.  
 Cathode current density: 3.5 amps./in.<sup>2</sup> initial calc.

|                               |           |      |      |      |      |
|-------------------------------|-----------|------|------|------|------|
| Screen Analysis:              |           |      |      |      |      |
| Size                          | +100      | +150 | +200 | +325 | -325 |
| Wt. %                         | 3.4       | 10.9 | 15.7 | 43.5 | 26.4 |
| Chem. Analysis, Wt. Percent W | 96.2      | 98.8 | 99.1 | 98.8 | 98.6 |
| Principal Impurity            | Fe, brick | Fe   | Fe   | Fe   | Fe   |
| X-ray Impurities              | None      | None | None | None | None |

continuing the flow until free chlorine gas is detected in the vented gas, the quality of the electrodeposit is maintained and the high recovery efficiency is sustained. This procedure is followed each day after the scheelite addition.

No scheelite or tungsten carbide was found in these samples. Iron is heaviest in +100 mesh, decreasing in the finer meshes to the lowest amount in -325 mesh. The iron is not in excess of 1/2%. Also molybdenum was below 0.01%.

TABLE III

Duration of Run: 4 hrs. each (2 runs mixed).  
 Temperature of Electrolysis: 1,000° C.  
 Bath Conc.: 9" depth, 6% by wt. calc. as W in  $\text{CaCl}_2$ .  
 Cathode: 2" dia. graphite 6" immersion.  
 Anode: Graphite cell pot.  
 Voltage: 2.2 volts.  
 Current: 150 amperes.  
 Cathode current density: 4.0 amps./in.<sup>2</sup> calc.

|                                 |           |      |           |      |      |
|---------------------------------|-----------|------|-----------|------|------|
| Screen Analysis:                |           |      |           |      |      |
| Size                            | +100      | +150 | +200      | +325 | -325 |
| Wt. %                           | 6.7       | 12.1 | 19.0      | 38.8 | 23.4 |
| Chem. Analysis W in Wt. Percent | 94.5      | 98.5 | 98.8      | 99.0 | 99.4 |
| Impurities                      | Brick, Fe | Fe   | Fe        | Fe   | Fe   |
| X-ray Analysis                  |           |      | Not Taken |      |      |

TABLE IV

Duration of Run: 4 hrs. each (2 runs mixed).  
 Temperature of Electrolysis: 1,000° C.  
 Bath Conc.: 10" depth, 2% by wt. calc. as W in  $\text{CaCl}_2$ .  
 Cathode: 2" dia. graphite, 7" immersion.  
 Anode: Graphite cell pot.  
 Cathode current density: 4.1 amps./in.<sup>2</sup> calc.  
 Voltage: 2.2 volts.  
 Current: 180 amperes.

| Screen Analysis:                | +100      | +150 | +200 | +325 | -325 |
|---------------------------------|-----------|------|------|------|------|
| Size                            | 1.1       | 7.8  | 17.2 | 55.9 | 18.0 |
| Wt. %                           |           |      |      |      |      |
| Chem. Analysis W in Wt. Percent | 93.4      | 98.4 | 98.9 | 99.0 | 98.7 |
| Principal Impurity              | Brick, Fe | Fe   | Fe   | Fe   | Fe   |
| X-ray Analysis                  | Not Taken |      |      |      |      |

Although the scheelite concentrate used in the feed contained 4.5 wt. percent Fe and 3.5% Mo, for some reason the cleaned electrodeposite from a regulated bath contained less than 0.25% Fe and less than .01% Mo. A possible explanation is that a  $\text{CaCl}_2$  electrolyte bearing about 10% by wt. of solute calculated as W "salts out" or precipitates  $\text{CaMoO}_4$  so that very little of any of the

15 The above mentioned apparatus was used to electrodeposit molybdenum from crude  $\text{CaMoO}_4$ . This crude feed was provided by roasting molybdenite ( $\text{MoS}_2$ ) concentrates in the common commercial fashion. The raw material contained 48% Mo (98%  $\text{CaMoO}_4$ ). The conditions of electrolysis were identical to those run for tungsten. The results are shown in Table V.

TABLE V

Duration of Run: 4 hrs. each (2 runs mixed).  
 Temperature of Electrolysis: 1,000° C.  
 Bath Conc.: 10" depth, 10% by wt. calc. as Mo in  $\text{CaCl}_2$ .  
 Cathode: 2" dia. x 7" immersion.  
 Anode: 10" graphite pot.  
 Voltage: 2.2 volts.  
 Current: 160 amperes.  
 Cathode current density: 3.5 amps./in.<sup>2</sup> initial calc.

| Screen Analysis:       | +100 | +150 | +200 | +325 | -325 |
|------------------------|------|------|------|------|------|
| Size                   | 2.0  | 15.6 | 32.7 | 40.6 | 9.1  |
| Wt. %                  |      |      |      |      |      |
| Principal Impurity, Fe | 2.1  | 2.7  | 2.2  | 2.7  | 3.0  |

molybdenum is available for electrolysis. There is no 35 question that the impurities are found in the sludge which forms in the bottom of the bath. The use of chlorine promotes the separation.

In a freshly prepared bath, the chlorine treatment speeds the time when the deposit fulfills required specifications. 40 Otherwise the first deposits are usually discarded. The purity of the deposit improves with the age of the bath. However, after prolonged use the impurities build up in volume so that it becomes difficult not to physically entrain impurities despite the chlorine treatment. At 45 this point it is practical to ladle out the insolubles or start anew.

The preferred cathode material is graphite, but other inert electrical conductors may be used.

Although the large bulk of the market is for 98.8% W, where a product whose purity is over 99.99% W is required, the tungsten hereinabove described may be electrorefined using the electrorefining method described in my Patent No. 2,960,451 or treated in the following way.

The electrodeposit stripped in accordance with the foregoing procedure is fed to a cell adequately covered, airtight and under inert gas pressure where it serves as anode. An inert cathode is immersed in the electrolyte for electrorefining of the tungsten. The preferred electrolyte is a 50-50 mol percent  $\text{NaCl} = \text{KCl}$  solvent containing 3-5% wt. percent  $\text{WCl}_3$ . The  $\text{WCl}_3$  solute is easily generated within the cell by bubbling  $\text{Cl}_2$  through the bed of tungsten resting on the bottom of the cell. The anode current density is preferably below 10 amps./in.<sup>2</sup> and 1-3 amps./in.<sup>2</sup> is adequate. The cathode current density may be varied widely with good results from a few tenths of an ampere per sq. in. to over 35 amps./in.<sup>2</sup>. The preferred cathode current density is in the range of 3-10 amps./in.<sup>2</sup>. The temperature of electrolysis is 750-800° C. The cathode and its electrodeposit are preferably cooled in an inert atmosphere. The adherent salts are readily washed away in water.

The tungsten metal crystals are macroscopic, silvery white, ductile and of extraordinarily high purity in excess 75 of 99.99%.

35 The molybdenum metal deposited was silvery bright in color and free from carbides, lower oxides, and the like. The iron content of the deposit was high due to the corrosion of the pot lining, the corrosion products falling into the bath. Normally, unless the bath is treated with chlorine gas prior to electrolysis, the first deposits are not as pure as subsequent deposits. The Mo in this example analyzed 97.0% for the reasons given.

In order to provide an electrolyte capable of producing molybdenum consistently having a purity in a bulk sample of 99.5% and selected crystals of 99.9%, chlorine gas is bubbled through the electrolyte of the foregoing runs set forth in Table V until free chlorine is detected in the effluent gas stream. Also, as in connection with the tungsten, molybdenum may be used as an anode in an electrorefining process similar to the one used in connection with the electrorefining of tungsten to produce a pure molybdenum metal. Similarly, as in the case of tungsten, a molybdenum chloride is formed in the electrolyte which is preferably of about five weight percent.

50 The scope of the invention as described in the foregoing is set forth in the appended claims.

I claim:

1. In a process for the continuous production of tungsten metal in excess of 99% purity by the fusion electrolysis of 55 scheelite concentrates added to a calcium chloride electrolyte, the improvement comprising controlling the composition of said electrolyte by bubbling chlorine gas through said electrolyte to convert to calcium chloride the calcium oxide released by the deposition of tungsten, thereby maintaining the high quality production of tungsten at a high recovery efficiency.

2. A continuous process for the electrolytic production of a refractory metal of the group tungsten and molybdenum comprising providing a molten electrolyte composed of the group of alkaline earth metal halides and at least one oxide of the group of alkaline earth metal oxides in substantial amount in said electrolyte, adding an oxide ore of said refractory metal including an oxide of the group of alkaline earth metals to maintain the desired amount of alkaline metal oxide in the electrolyte, electrolyzing the said molten electrolyte between an anode

and cathode for depositing said refractory metal in pure, ductile and large crystalline form on a cathode immersed in the electrolyte and adding chlorine to convert to alkaline earth metal chloride the oxide of the alkaline earth metal released by the deposition of the refractory metal, thereby maintaining the electrolyte at a high recovery efficiency.

3. A continuous process for the electrolytic production of a refractory metal of the group tungsten and molybdenum as set forth in claim 2 wherein said alkaline earth halide is calcium chloride and said oxide ore is a scheelite concentrate for the production of pure ductile tungsten in large crystalline form.

4. A continuous process for the electrolytic production of a refractory metal of the group tungsten and molybdenum as forth in claim 2 wherein said refractory metal is molybdenum and said alkaline earth halide is calcium chloride.

5. In a process for the continuous production of molybdenum metal in excess of 99% purity by the fusion

15

10

20

electrolysis of calcium molybdenum oxide concentrates added to a calcium chloride electrolyte, the improvement comprising controlling the composition of said electrolyte by bubbling chlorine gas through said electrolyte to convert to calcium chloride the calcium oxide released by the deposition of molybdenum, thereby maintaining the high quality production of molybdenum at a high recovery efficiency.

6. In a process for the production of tungsten metal as set forth in claim 1 wherein the said composition of said electrolyte is maintained between about 0.1% and 15% free calcium oxide.

References Cited by the Examiner

UNITED STATES PATENTS

2,960,451 11/1960 Slatin ----- 204-64

JOHN H. MACK, *Primary Examiner.*

H. S. WILLIAMS, *Assistant Examiner.*